

T. W. CAVERS.  
SMELTING LEAD AND LIKE ORES AND PRODUCTS.  
APPLICATION FILED AUG. 9, 1918.  
1,343,656. Patented June 15, 1920.



Inventor

T. W. Cavers

By A. B. Fatty, Attorney

# UNITED STATES PATENT OFFICE.

THOMAS W. CAVERS, OF COPPERHILL, TENNESSEE, ASSIGNOR TO GARRED-CAVERS CORPORATION, OF NEW YORK, N. Y., A CORPORATION OF NEW YORK.

## SMEILING LEAD AND LIKE ORES AND PRODUCTS.

1,343,656.

Specification of Letter's Patent. Patented June 15 1920.

Application filed August 9, 1918. Serial No. 249,199.

To all whom it may concern:

Be it known that I, THOMAS WILLARD CAVERS, a subject of the King of Great Britain, residing at Copperhill, in the county of Polk and State of Tennessee, have invented certain new and useful Improvements in Smelting Lead and like Ores and Products, of which the following is a specification.

10 The present invention has for its object to produce economies in the smelting of lead ores and products, or lead ores or products (whether or not they contain other base metals or precious metals or both), which 15 operation is ordinarily carried out in a water-jacketed blast furnace.

In the ordinary process, lead ores and products, such as roasted lead sulfid or galena, together with a flux such as limestone and silicious matter is introduced into the upper part of the blast furnace, together with more or less coke. In the ordinary methods of operating, the amount of coke necessary will depend to a considerable extent upon the character of the ore and other conditions, and in practice a minimum quantity of coke relative to the burden in the furnace is employed. The ore is usually roasted or otherwise treated to eliminate most of the sulfur and the lead is largely in the form of an oxid and is reduced by the carbon of the coke in the charge fed at the top of the furnace. The silicious material and the limestone flux, together with the iron, combine to form slag and a certain amount of matte or speiss is made, depending upon the condition of the charge and the amounts of sulfur and arsenic present. To produce the above reactions, heat is necessary and this has heretofore all been supplied by the addition of coke with the ores and fluxes at the top of the furnace. There is an excess of coke added to the charge, over and above the quantity necessary to reduce the lead oxid to metallic lead, and this excess coke is burned in the lower part of the furnace by the oxygen in the blast, which is introduced into the furnace through the twyters. The burning of this excess coke provides the heat to keep the slags molten and maintain the temperature at which the reactions in the furnace take place.

In other kinds of metallurgical operations it has been proposed to blast in fuel. This has been proposed in connection with numerous reducing processes in which iron oxid ore, or oxidized iron ore, is mixed with reducing agent and flux, and heated under reducing conditions for the purpose of producing iron metal. It has also been proposed to introduce fuel with the blast through the twyters in the smelting of copper and like ores, in which the heat required for smelting is produced, partly by oxidation of the sulfur and iron in the charge, and partly, by the burning of carbonaceous material introduced into the furnace through the twyters with the blast, (see my U. S. Patent 1,259,467).

According to the present invention I introduce, with the blast in the lower part of the furnace, a short distance above the normal slag level therein, fine coal, or other carbonaceous fuel, but only for the purpose of supplying the heat to maintain the reaction temperature in the furnace, by uniting with the oxygen of the blast, which fuel will then take the place of the excess coke added with the charge at the top of the furnace in ordinary practice, and in this way effect an economy in the smelting of lead. Only enough coke, according to the present invention, need be added with the charge at the top of the furnace to effect the reduction of the oxid of the easily reducible metals, such as lead. It is not necessary to previously coke the coal to be introduced with the blast at the twyters, but this coal may be and preferably is employed in its original (uncoked) condition, usually as a fine powder, for example, cheap soft coal, dried and pulverized.

In addition to coal, I may add in this manner other lead-bearing material, lead-bearing flue dust, finely divided ores carrying base or precious metals, and in some cases I may also employ fluxing agents. This is, of course, in addition to the material introduced at the top of the furnace.

In some instances it is possible to employ other kinds of carbonaceous fuel, oil in some instances being suitable, and this likewise may be mixed with flue dust, ore material and the like.

In the accompanying drawing, forming a

part of the present specification, I have illustrated apparatus suitable for use in carrying out the process of my present invention, the view being a vertical elevation, 5 parts being shown in section.

In said drawing, 1 represents a blast furnace of the water-jacketed type, 2 the sole plate, 3 suitable supports, and 4 one of the twyers, of which there may be any suitable 10 number. The dotted line 5 represents the normal slag level. 6 is the bustle pipe and 7 the twyer pipe, in which the blast is regulated by the gate or valve 8. Into some 15 point in the air passage, and preferably between the gate 8 and the twyer box 4 is connected a fuel supply pipe 9 leading from a hopper-bottomed receptacle or bin for introducing the coal, with or without the other materials above referred to. In the bottom 20 of this receptacle or bin, I place a screw conveyor, the end of which enters the upper end of pipe 9 as shown at 11, which is suitably revolved, as by gear 12. The screw will keep the upper and horizontal end of the 25 pipe filled with coal, which will prevent air from blowing out through the bin 10. Other means may be employed to prevent air from the twyer pipe blowing back through the coal pipe and bin.

In operation, coal, *e. g.* fine soft coal, coal slack, or in some instances coke breeze, etc., preferably crushed and pulverized, to which may be added the materials above referred to, is fed by the screw 11, into pipe 30 9, the end of the screw and the fine material in the convolutions thereof within the pipe 9 forming an air seal, then the said material flows downwardly through the sloping part of pipe 9, into the twyer pipe 7, where it is 35 rapidly carried by the blast into the furnace, where the coal, etc., is practically all burned in the slag-forming zone.

In the réduction of iron ores in the blast furnace, it has heretofore been proposed 40 to blast in coal or other carbonaceous material, for furnishing the reducing agent necessary to reduce the oxids to metal. I make no claim to the introduction of fuel or any other material with the blast for the 45 purpose of reducing the metal, but only to produce the heat necessary to maintain the temperature at which the proper reactions will take place in the blast furnace, which heat has, in practice heretofore, been supplied by the burning of the excess coke added to the charge, by the oxygen of the blast air. "Excess coke" may be defined as that charged to the furnace in excess of the 50 amount theoretically necessary for the reduction of metals such as lead.

In smelting, according to the present invention, I am able to secure certain advantages, namely, I am able to employ low grade fuel, that is to say, cheap fuel in the 55 form of soft coal and the like, and if de-

sired, I can also introduce other materials, such as those above referred to, with the blast. The amount of coke that need be used, is materially less than that necessary for smelting in the ordinary way, and coal, 70 a much cheaper material, is substituted for the coke so dispensed with.

In the smelting of ordinary grades of lead ores, by the old process it has been customary to employ about 12 to 15% of coke 75 based upon the weight of the charge in the furnace. In accordance with the present invention, I would add to the furnace charge containing such grades of ore about 9 to 12% of coke, and the amount of fine coal 80 or similar fuel blown in through the twyers would amount to about 2 to 3% of the weight of the charge. These proportions, of course, are subject to more or less variation, depending upon the nature of the particular 85 ore, flux and furnace conditions.

What I claim is:—

1. A process of smelting oxidized lead ores or other lead-containing materials, which comprises the step of heating a mixture of lead oxid material and carbonaceous reducing agent, by means of the combustion of powdered coal introduced into the furnace with an air blast.

2. A process which comprises blowing into 95 a blast furnace containing a mixture of lead oxid material and coke in amount sufficient to reduce the same, a blast of air carrying fine carbonaceous fuel, the amount of such air being not greatly in excess of the quantity necessary to burn said fine carbonaceous fuel so introduced, whereby the coke reduces the lead oxid, and the air and fuel blown in furnishes the heat necessary to promote the reaction.

3. In the blast furnace smelting of lead ores, the step of heating the charge essentially by blasting in carbonaceous fuel with air to burn the same, into the lower part of the furnace above the normal slag level 100 therein, the amount of such coal being sufficient to maintain reducing conditions.

4. In the process of smelting in a blast furnace, lead-bearing ores or products, the step of introducing carbonaceous fuel with the blast to supply the heat necessary to produce such a temperature in the lower part of the furnace, continuously, as will maintain the reactions between the coke and the oxids of lead and between the silica and the iron and lime, the said carbonaceous fuel being burned in the lower part of the furnace and the coke being consumed in the reaction between the carbon it contains and the oxids of lead.

5. A process of smelting lead ores and products to produce metallic lead, which may also carry other base metals and precious metals, which process comprises the step of introducing a relatively small amount of 110

carbonaceous fuel as fines, with the blast, into the lower part of the furnace at a point somewhat above the slag level, where the coal so introduced is practically all consumed, whereby the quantity of coke introduced at the top of the furnace with the

charge may be cut down substantially to that necessary to react with the lead and other oxids present to reduce the same to the metallic state. 10

In testimony whereof I affix my signature.  
THOMAS W. CAVERS.